

## UNITED STATES PATENT OFFICE

2,320,028

CONVERTING PHOTOGRAPHIC IMAGES  
INTO COLOR

Percy D. Brewster, Holmdel, N. J.

No Drawing. Application July 3, 1940,  
Serial No. 343,747

7 Claims. (Cl. 95—88)

This invention relates to color photography, more particularly to the converting of silver photographic images carried by a gelatin coating on a suitable support into a dye mordant, which, when treated with the proper dyes forms images in color.

The chief object of the invention, stated generally, is the conversion of positive silver images, printed from a negative, into a silver iodide mordant of adequate dye-absorptive power which is relatively or totally transparent to transmitted light, and which, when dyed, reproduces the original negative silver grain complexes in color to a marked extent. A further object is the quick conversion of long lengths of cinematographic film into a dye mordant of uniform dye absorbing power at low cost. Another object is the complete conversion of the silver images into colloid or gel form of silver iodide. To these and other ends my invention comprises the novel features hereinafter described.

Silver iodide mordants have been formed by several different methods producing different types of mordant, each having well defined characteristics, for example; Traube in United States Patent No. 1,093,503, dated April 14, 1914, hereinafter referred to as the "Traube type," produces a translucent white or yellowish-white mordant that absorbs dye very slowly to produce dull images, unsuited for modern color cinematography, but which reproduces the negative image grain or grain complexes with extreme accuracy. Miller in United States Patent No. 1,214,940 dated February 6, 1917, hereinafter referred to as the "Miller type," produces, under proper processing conditions, a mordant that is absolutely transparent to the eye to transmitted light and that adsorbs dye strongly and quickly to produce brilliant images but reproduces the negative image grain or grain complexes comparatively poorly, especially in the highlights. In my United States Patent No. 1,992,169 dated February 26, 1935, hereinafter referred to as "1935 Brewster type," I formed the mordant by action of a gaseous acid producing a mordant, which, under proper processing, produces a transparent mordant which adsorbs dye quickly to produce a brilliant image closely resembling the "Miller process" mordant but reproducing the negative image grain or grain complexes much more sharply though probably not equalling the sharpness of the "Traube process."

If the "Traube type" mordant is formed, as is usual, without using one of the metallic salts of the iodides in the reaction, I believe to the best

of my present chemical knowledge, the mordant formed is a pure crystalloid consisting of silver iodide. The "Miller type" mordant, formed under ideal conditions is fully transparent and probably is a colloid, the gel of silver iodide, but if the mordant is of the thin whitish translucent type, I believe it consists of a mixture of the crystalloid and colloid forms of silver iodide. The mordant formed by the "1935 Brewster type" under ideal conditions is transparent, adsorbs dye very well and produces sharp images but, in practice, requires a careful control of the pH of the "soak" solution to produce even results over long lengths of film and is not adapted for the production of a heavy translucent mordant to yield dull color images or sound track.

This invention in general comprises impregnating the gelatin coating bearing silver images, with a solvent for iodine or other suitable bleach and then subjecting the impregnated coating to iodine or other suitable bleach in gaseous or vapor form. Solvents may consist of iodides such as potassium or sodium iodide or glacial acetic acid or certain alcohols diluted with water. The effectiveness of many of these solvents may be increased if the solvent is acidified. The bleach may be iodine vapor or gas containing iodine vapor or hydriodic acid in gaseous form. The mordant so formed in the gelatin may be treated with a reducing agent for example: a two percent solution of sodium-bisulphite to clear it of excess iodine and may then be dyed in the usual manner.

For most purposes in color cinematography, except production of sound track, I prefer to form a mordant which is transparent or which has only a thick, whitish, translucent "ghost" image which absorbs dye strongly and quickly and which when dyed reproduces the silver image grains or grain complexes with the greatest accuracy.

To accomplish this I prefer to use iodine vapor at a temperature not much above room temperature and a solvent impregnated in the gelatin coating which not only freely dissolves the iodine vapor but has a strong tendency to form a colloidal gel of silver iodide. The metallic salts of the iodides possess this quality, especially potassium iodide, which I prefer to use for the solvent in a relatively weak solution. I believe, to the best of my present chemical knowledge, that transparent colloidal silver iodide mols, especially those forming the weak portions of the image, are dissolved by the action of strong iodides used as solvents within the gelatin causing the sharp

outlines of the silver image grain complexes to be dissolved out or causing them to diffuse resulting in loss of definition of the mordant image. For example, using hardened gelatin, 5% to 8% solutions of potassium iodide have little or no solvent action on the silver image or mordant in the short time the solvent is necessarily in contact with the mordants but if stronger potassium iodide is used it is possible under certain conditions, that the sharpness of the images may be affected.

It is impossible to offer a fixed formula for "bleaching" or converting the silver image into a mordant adapted for color cinematographic use under all conditions. The kind of gelatin used, the type of the silver halide, the development, density of the silver image, whether gelatin is hardened, humidity in the gas chamber, etc., are factors to be considered in determining strength of solvent or concentration of gas. This process has a very wide latitude permitting very considerable changes in formulae without showing appreciable changes in the finished picture.

This process intensifies strongly, so I prefer a positive film with the images developed to a low contrast or gamma and which has been hardened in a formaldehyde solution and dried without rinsing, though good results can be obtained on unhardened film.

At present I prefer, in the practise of my invention, to use iodine gas or vapor to convert the silver images into dye mordants. Iodine vapor is much heavier than air and is readily formed by placing iodine in a vessel or chamber and circulating air over it, the strength of the iodine vapor being largely controlled by the temperature of the air in contact with it. The gelatin coating, bearing the silver images to be bleached, may be impregnated with a 7½% solution of potassium iodide, a ten to thirty second immersion being usually sufficient. The excess solution is removed from the gelatin surface by an air blast or squeegee. The film is then treated with the iodine gas in a chamber at a temperature of about 73 degrees F. until the silver images are converted or bleached into the mordant, and quickly cleared in 3% sodium bisulfite solution and rinsed. The time of bleaching may vary from thirty to ninety seconds under ideal conditions. It is to be understood that the concentration of the potassium iodide and iodine vapor and time of treatment may vary to any extent without departing from my invention. Speaking generally, if the iodine vapor is too concentrated there is a tendency to bleach quickly and to form the "Traube" type of mordant, while too weak an iodine vapor may cause a slow bleach which forms a whitish mordant that may not dye so well.

A weak potassium iodide solution has some advantages. It may not have sufficient iodide present to form the best colloidal mordant and may cause a slow bleach, while too strong an iodide solution, to the best of my present knowledge, may have a solvent action on the mordant and cause a loss of image sharpness. If the concentration of the iodide be sufficiently high, the gelatin, especially if it is not hardened, may be dissolved. Images can be bleached with a 1% solution of potassium iodide but the operation is slow and little advantage seems to be gained.

If sound tracks are being colored or intensified I prefer a more opaque "Traube type" image and do not require a gel forming salt or only a very small amount of such salt in the solvent.

To form the opaque mordant of the "Traube type," I prefer to use a higher vapor pressure of iodine at a temperature of one hundred degrees F. or more in a combination with a solvent which is weak in iodide or contains no iodide at all. Such a combination produces an extremely rapid bleach probably tending to reduce the formation of colloid or gel form of iodide and results in a heavy mordant.

10 Compounds of iodine in gaseous form may be substituted for free iodine in the bleach chamber such for example as—hydrogen iodide (hydroiodic acid). In such case the gelatin coating must be impregnated with acidified solvents 15 which I believe cause iodine to be liberated from the hydrogen iodide. The mordant so formed will be of the opaque "Traube type" unless the solvent also includes a gel forming salt such as potassium iodide in which latter case a more completely transparent mordant may be formed. The hydrogen iodide gas may be mixed with air or other gas to control the speed of the reaction.

The alkali metal iodides such as ammonium or sodium iodide may be substituted for potassium iodide. Many of the metallic iodides such as 25 cadmium iodide are solvents of iodine vapor and cause the gelatin coating, when treated with iodine vapor, to become discolored with the reddish brown iodine stains, but the penetration of 30 the iodine into the gelatin is usually quite slow and an unsatisfactory mordant results unless a colloid forming salt is present.

"Impregnating" the gelatin coating with a solvent is intended to mean thoroughly moistening but not necessarily saturating the gelatin 35 with the solvent.

The "solvent" in the gelatin for iodine vapor does not imply any chemical reaction. However, when hydrogen iodide is used as a bleaching 40 agent the acidified solvent causes free iodine to be liberated which may be dissolved and carried into the gelatin by the iodide present in the solvent which also results in the formation of a transparent gel mordant.

45 I claim:

1. Process for converting a silver photographic image carried in a gelatin coating on a suitable support into a transparent dye mordant without substantial loss of definition which comprises 50 impregnating said coating with a solvent for a gaseous bleach then treating said coating with said gaseous bleach.

2. Process for converting a silver photographic image carried in a gelatin coating on a suitable support into a transparent dye mordant without substantial loss of definition which comprises 55 impregnating said coating with an acidified solvent for a gaseous bleach then treating said coating with said gaseous bleach.

3. Process for converting a silver photographic image carried in a gelatin coating on a suitable support into a transparent dye mordant without substantial loss of definition which comprises 60 impregnating said coating with a solvent for iodine vapor then treating said coating with gas containing iodine vapor.

4. Process for converting a silver photographic image carried in a gelatin coating on a suitable support into a transparent dye mordant without substantial loss of definition which comprises 65 impregnating said coating with a solution of potassium iodide and treating said coating with iodine vapor.

5. Process for converting a silver photographic image carried in a gelatin coating on a suitable

support into a transparent dye mordant without substantial loss of definition which comprises impregnating said coating with an acidified solvent for hydrogen iodide and treating said impregnated coating with gaseous hydrogen iodide.

6. Process for converting a silver photographic image carried in a gelatin coating on a suitable support into a transparent dye mordant without substantial loss of definition which comprises impregnating said coating with an acidified solution of potassium iodide and treating said im-

regnated coating with a gas containing hydrogen iodide.

7. Process for converting a silver photographic image carried in a gelatin coating on a suitable support into a dye mordant which comprises impregnating the said coating with an acidified solvent for a gaseous bleach and treating said coating with said gaseous bleach and controlling the solvent and bleach so as to form either a

10 transparent or opaque mordant.

PERCY D. BREWSTER.